

# UNITED STATES PATENT OFFICE.

HENRY BENJAMIN, OF MONTREAL, CANADA, ASSIGNOR OF ONE-HALF TO  
FREDERICK B. WELLS, OF SAME PLACE.

## COMPOSITION FOR ROADWAYS, &c.

SPECIFICATION forming part of Letters Patent No. 443,953, dated December 30, 1890.

Application filed February 5, 1890. Serial No. 339,227. (No specimens.)

*To all whom it may concern.*

Be it known that I, HENRY BENJAMIN, of the city of Montreal, in the district of Montreal and Province of Quebec, Canada, have 5 invented a new and Improved Composition for Roadways, Fire-Proof Roofing, and other Building Purposes, of which the following is a full, clear, and exact description.

My invention consists of a composition of 10 matter, mainly designed for roadways, sidewalks, fire-proof roofing, vault-linings, and various building and other purposes, the same having for its ingredients finely-divided iron particles and a bituminous substance, sub- 15 stantially as hereinafter described.

I take, for instance, finely-divided particles of iron or iron ore—such as the waste products from iron mines or iron sand—and mix the same with a bituminous substance, such as ordinary natural asphalt or the asphalt of commerce, or other equivalent material possessing like qualities and serving as a matrix for the iron particles. These ingredients are to be thoroughly mixed and incorporated together 20 by heat to bring the mass to a plastic or pasty consistency, and are usually designed to be applied while hot to the surface which the composition is intended to cover, the covering or coating thus applied being of any de- 25 sired thickness, according to the requirement of the work. Rollers or any other suitable pressure means may be employed in laying down roadways and sidewalks with the composition; and in the case of roofing and vault- 30 linings the composition may be floated on.

In using this composition on roofs I prefer to add a finely-pulverized coating of ground plumbago or mica, so as to render it entirely fire-proof.

The composition when reduced to a semi- 40 liquid condition may be used for grouting between stone or wooden paving-blocks for street-roadways. When pressed into blocks it can be very durably and advantageously employed in submarine works, such as bridge- 45 piers, and also for other building purposes.

It will be impossible for me to confine myself to any exact relative proportions of the ingredients named, but the following statement will serve to explain what variations 50 may be made. Thus when great resistance is required—as, for instance, when the composition is used for a roadway subjected to heavy traffic, the proportion of the iron particles may be the largest; but in such case I 55 prefer to use about equal quantities, or thereabout, by weight, of the iron particles and the bitumen of commerce. If, however, I use the genuine natural asphalt, such as that known as "Swiss," "Cuban," "Mexican," or 60 "African," a much smaller proportion of the bitumen will be needed.

When using natural bitumen, I add to it to give it the necessary plasticity a small quantity of pitch or petroleum residuum when 65 mixing.

Having thus described my invention, what I claim as new, and desire to secure by Letters Patent, is—

The herein-described composition of matter, consisting in waste granular or fragmentary iron ore and asphaltum or bitumen, sub- 70 stantially as described.

HENRY BENJAMIN.

Witnesses:

F. B. MCNAMEE,  
W. G. TURNER.